

1

2,906,443

## WAX COMPOSITIONS

Waldon T. Harvey, Hockessin, Del., and Seymour W. Ferris, Mount Holly, N.J., assignors to Sun Oil Company, Philadelphia, Pa., a corporation of New Jersey

No Drawing. Application February 4, 1958  
Serial No. 713,089

4 Claims. (Cl. 229—3.1)

This invention relates to a new wax composition especially suitable for coating fibrous containers such as milk containers.

Paraffin waxes have heretofore been employed for coating paper containers designed to hold liquids, but such waxes suffer many shortcomings. In order to overcome some of the difficulties, microcrystalline waxes and polymers, such as polyethylene, have been incorporated therewith. Such compositions, however, have also been unsatisfactory in that containers coated therewith suffer one or more of the following difficulties: in presenting an unsightly appearance, in obtaining poor coverage with subsequent softening when filled with liquids, in blocking at relatively low temperatures, in easily fracturing on being subjected to an impact, and in requiring conditions during application to paper containers which cannot be met with existing equipment, such as relatively high temperatures. For example, United States Patent Number 2,624,501 describes and claims a paraffin wax which is especially suitable for coating fibrous sheet materials and containers such as milk containers. However, actual commercial use has disclosed several disadvantages of coatings formed from this wax. Such coatings on fibrous sheet materials may develop minute imperfections which impart a serpentine effect to the coating thereby creating an unsightly appearance and leakage of packaged liquid materials through the imperfections may develop. A further difficulty of this wax, as has been found, is the tendency of coatings formed therefrom to fracture on suffering an impact so that leaks develop through the fracture.

An object of the present invention is to provide a wax composition especially suitable for coating fibrous containers for fluids. A particular object is to provide a wax composition effective for coating paper containers for liquids which imparts a pleasing appearance to the resulting article of manufacture, while obtaining good coverage and good blocking characteristics, and which can be readily applied with existing equipment. A further object is to provide a process for the preparation of such wax compositions. A specific object is to provide a wax composition which, when formed as a coating for a fibrous container, will not easily fracture on suffering an impact.

It has now been found that by blending two paraffin waxes having specific properties in specific proportions, a wax composition achieving the above and other objects is obtained.

As used herein, melting points are determined by ASTM D87-42, penetrations by ASTM D5-52 and viscosities (SUS—Saybolt Universal Seconds) by ASTM D446-53, unless otherwise stated. Modulus of rupture, which is a measure of the tendency of the wax to fracture on suffering an impact, which may be in the form of a sharp impact or a continuous pressure, is determined by forming a wax into strips of specified dimensions (0.15 inch thick by 0.5 inch wide by 3 inches long) by solidifying molten wax on the surface of water to form the de-

2

sired thickness, and cutting to the other dimensions. Each strip is placed upon two horizontal supports two inches apart and is broken by incremental weighting at the center, the test being made at a temperature of 73° F. 5 The breaking weight in p.s.i. (pounds per square inch) of cross sectional area is the modulus of rupture.

The first paraffin wax must have a melting point of from 125° F. to 130° F., a penetration (at 77° F.) of from 17 to 23 (about 100 at 100° F.), a viscosity (at 210° F.) of from 36 to 39 SUS and a modulus of rupture (at 73° F.) of about 270 to 340. A paraffin wax meeting these specifications may be prepared by two methods. In the first method of preparing the described paraffin wax, a slack wax from the dewaxing of lubricating oil, 15 which may contain about 30% oil, is vacuum distilled and the fraction distilling between about 390 and 565° F. at 2 mm. of mercury pressure is collected. This fraction is dissolved in a solvent, preferably a mixture of methyl ethyl ketone and benzene in about equal volumes. Dissolution is performed at an elevated temperature, from about 165° F. to 195° F. being suitable, and advantageously about 6 parts by volume of solvent per part of wax is used. The solution is slowly cooled to a temperature of from 75° F. to 83° F. and the wax which 20 precipitates at this temperature is separated such as by filtration. The solution separated from the precipitated wax is further slowly cooled to a temperature of from 28° F. to 33° F. and the wax which precipitates at this temperature is separated and forms the first paraffinic 25 wax of the present compositions. Preferably the wax after separation from solution is washed such as with the solvent employed for dissolution, preferably at the same temperature as used for filtration, namely from 28° F. to 32° F., and the wax is then separated.

An alternate method of preparing the first paraffin wax of the present invention which provides considerable flexibility in obtaining the desired wax product is to separate from slack wax two distillate fractions, one distilling in the range of from about 390° F. to 475° F. at 2 40 mm. of mercury pressure and a second fraction distilling in the range of from about 450° F. to 565° F. at 2 mm. of mercury pressure. As usually occurs, the initial boiling point of the second fraction will overlap the end point of the first-mentioned distilled fraction. The lower boiling distillate fraction is dissolved in a solvent as above described and the solution cooled to a temperature of from 25° F. to 31° F. The wax which precipitates at this 45 temperature is separated as by filtering. The higher boiling distillate fraction is dissolved in a solvent as above described, except that a lower proportion of solvent to wax, say about 4.5 parts of solvent per part of wax, is advantageously used, and the solution slowly cooled to a temperature of from 72° F. to 82° F. The wax which precipitates at this temperature is separated such as by filtering and the remaining solution is further slowly 50 cooled to a temperature of from 25° F. to 31° F. The wax which precipitates at this latter temperature is separated as by filtering. The two distillate waxes so-prepared are combined to form the first paraffin wax of the present invention. Considerable flexibility is obtained since the 55 blending may be in various proportions so that the properties of the resulting wax mixture is within the limits above-described for the first paraffin wax. If desired, the two waxes can be washed and dried prior to blending, or the wet waxes may be combined and simultaneously washed and then recovered by removal of the wash liquid. In 60 general, from about 69% to 75% by weight of the paraffin wax will consist of wax from the lower boiling distillate fraction since, as has been found, such mixture gives a wax having properties within those defined for the first paraffin wax of the invention.

The second paraffin wax of the invention must have a 65

The second paraffin wax of the invention must have a

melting point of from about 148° F. to 154° F., a penetration (at 100° F.) of from 13 to 19, a viscosity (at 210° F.) of from 40 to 46 SUS and a modulus of rupture of from about 340 to 400.

The second paraffin wax of the subject wax composition is preferably prepared from a slack wax from the dewaxing of lubricating oil or from topping a high wax content crude oil, distilling the reduced wax crude under vacuum, and collecting the fraction distilling in the range of from about 450° F. to 565° F. at 2 mm. of mercury pressure. The distillate fraction is dissolved in a solvent which is preferably a mixture of methyl ethyl ketone and benzene in about equal parts by volume, dissolution advantageously being at a temperature of from about 165° F. to 190° F. as above described, using about 2 parts of solvent per part of wax. The solution is slowly cooled to a temperature of from about 77° F. to 83° F. and the wax precipitated at this temperature is separated and the separated wax is washed such as with the solvent employed for dissolution, preferably at the same temperature as used for filtration, and the wax recovered. This wax forms the second paraffinic wax of the present invention.

In preparing the wax constituents of the subject paraffin wax composition, the described operating variables must be observed in order to secure the advantages of the invention. However, the solvent used for dissolution of the wax fractions can be varied somewhat and good results obtained. The described solvent, consisting of about equal parts by volume of methyl ethyl ketone and benzene gives good results, but more or less of the two constituents, say from 30% to 70% by volume of benzene can be used. Also, other solvents can replace, at least in part, either the methyl ethyl ketone or benzene. For example, toluene can be substituted for a portion of the benzene, and good results obtained.

The two paraffin waxes which form the wax composition of the present invention must be blended in specific proportions in order to obtain the advantages of the present invention. The first described paraffin wax forms from 70% to 85% of the composition, and the second paraffin is present in a quantity of from 30% to 15%. This blend, as shown hereinafter by example, has novel and unobvious properties including a remarkably high modulus of rupture, which is at least 420, and may be as high as 500, and is always at least 30 units higher than the modulus of rupture of either of the wax components of the composition. The blend has a melting point of from 130° F. to 132° F., a viscosity (at 210° F.) of from 38 to 41 SUS, and a penetration (at 100° F.) of from 50 to 80.

In order to demonstrate a specific embodiment of the present invention and the advantages thereof, two paraffin waxes were prepared as follows: slack wax from the dewaxing of lubricating oil and containing about 30% oil was distilled at a pressure of 2 mm. of mercury. A distillate fraction boiling in the range of from about 390° F. to 475° F. and another distillate fraction boiling in the range of from about 450° F. to 565° F. were collected. The lower boiling fraction was dissolved in a mixture of 60% methyl ethyl ketone and 40% benzene at an elevated temperature of about 170° F., about 6 parts of the solvent per part of wax being used. The solution was slowly cooled to 28° F. and the precipitated wax was filtered, washed and dried. The higher boiling distillate fraction was dissolved in a similar solvent as above described, using about 4.5 parts of solvent per part of wax, and the resulting solution cooled to 80° F. The wax precipitated was separated by filtering and the filtrate was further cooled to 30° F. The wax separating at this latter temperature was separated by filtering and was washed and dried. The two so-formed waxes were blended in quantities such that the final composition contained 72% of wax from the lower boiling distillate and 28% from the higher boiling distillate. The resulting wax product

had a melting point of 127° F., a viscosity (at 210° F.) of 39.0, a penetration (at 77° F.) of 20 and a modulus of rupture (at 73° F.) of about 338.

The second paraffin wax component of the present composition was prepared by topping a high wax content crude petroleum to about 38% bottoms. The bottoms were charged to a vacuum distillation operation operating at 2 mm. of mercury pressure, and the fraction distilling between 450 and 565° F. was collected. This fraction was dissolved in a solvent consisting of a mixture of about 60% methyl ethyl ketone and about 40% benzene at a temperature of about 180° F., about 2 parts of solvent per part of wax being used. The resulting solution was slowly cooled to 80° F. and the wax precipitated at this temperature was separated, washed and dried. This second paraffin wax had a melting point of 151° F., a viscosity (at 210° F.) of 43.6, a penetration (at 77° F.) of 12 and a modulus of rupture (at 73° F.) of 352.

Blends containing varying quantities of the two components were prepared by admixing the components at a temperature above their melting points to form a homogeneous product, and cooling. It was found that blends containing from 70% to 85% of the lower melting paraffin wax, the remainder of the composition being the higher melting paraffin wax, exhibit a synergistic effect in that the modulus of rupture is far above that which would be expected on blending the two components. Results obtained are shown in the following table:

| 30 | 1st wax, weight percent | 2nd wax, weight percent | Modulus of rupture, p.s.i. of cross sectional area |
|----|-------------------------|-------------------------|----------------------------------------------------|
| 35 | 0.....                  | 100                     | 352                                                |
|    | 25.....                 | 75                      | 400                                                |
|    | 50.....                 | 50                      | 400                                                |
|    | 75.....                 | 25                      | 445                                                |
|    | 82.....                 | 18                      | 432                                                |
|    | 90.....                 | 10                      | 385                                                |
| 40 | 100.....                | 0                       | 338                                                |

Milk containers formed from cardboard were coated with the wax composition in a commercial operation using existing equipment. No difficulties such as fouling of the equipment with solidified or partially solidified wax were observed. The coated container exhibited a high gloss with no serpentine effects. Good coverage is obtained and no fracturing is observed on subjecting the coated containers to impacts designed to be more severe than impacts received in service, and blocking of the containers when stored in contact with each other at temperatures as high as 100° F. is not observed. Also, blocking of slabs formed from the subject wax composition and stored in contact with each other is not observed at temperatures of about 100° F.

It does not appear that other waxes can be substituted for either component of the present composition without changing one or more properties of the resulting compositions so that the objects of the present invention are defeated. For example, a paraffin wax having a melting point of 142° F., a viscosity of 40 (SUS at 210° F.) a penetration (at 77° F.) of 12 and a modulus of rupture of 324 when substituted for the higher melting paraffin wax of the present composition gave a blend in which the modulus of rupture showed no synergism. The substitution of still other waxes having closely related properties but lying outside of those defined for the two components of the present compositions were made, none of which were operative in providing all of the advantages of the present compositions.

70 The invention claimed is:

1: A wax composition consisting essentially of from 70% to 85% of a paraffin wax having a melting point of from 125° F. to 132° F., a penetration at 77° F. of from 17 to 23, a viscosity at 210° F. of from 36 to 39 SUS and a modulus of rupture at 73° F. of from about 270 to

340, and from 15% to 30% of a paraffin wax having a melting point of from 148° F. to 154° F., a penetration at 100° F. of from 13 to 19, a viscosity at 210° F. of from 40 to 46 SUS, and a modulus of rupture of from about 340 to 400.

2. A wax composition according to claim 1 wherein the modulus of rupture is at least 30 units higher than the modulus of rupture of the individual wax components.

3. A container for holding liquids formed from a fibrous sheet material and provided with an adherent moisture and liquid resistant coating, said coating being formed from the wax composition of claim 1.

4. A new composition of matter consisting essentially

of paraffin waxes, said composition having a melting point of from 130° F. to 132° F., a viscosity at 210° F. of from 38 to 41 SUS, a penetration at 100° F. of from 50 to 80, and a modulus of rupture of from about 420 to 500, the modulus of rupture being at least 30 units higher than the modulus of rupture of the paraffin wax components.

**References Cited in the file of this patent**

**UNITED STATES PATENTS**

|           |                     |               |
|-----------|---------------------|---------------|
| 2,467,959 | Bowman et al. ----- | Apr. 19, 1949 |
| 2,756,180 | Perry et al. -----  | July 24, 1956 |